

## UNITED STATES PATENT OFFICE

2,671,737

## ALUMINUM COATING PROCESS AND FLUX

Walter E. Jominy, Detroit, and John H. Olson,  
Berkley, Mich., assignors to Chrysler Corpora-  
tion, Highland Park, Mich., a corporation of  
Delaware

No Drawing. Application October 10, 1950,  
Serial No. 189,478

6 Claims. (Cl. 117—51)

1

This invention relates to improvements in the formation of aluminum and aluminum alloy coatings on steel and more particularly to an improved process and flux for forming an integral type bond between aluminum or aluminum alloy and steel.

One of the main objects of the invention is to provide a flux of this kind which may be applied to the steel to be aluminum coated in the form of a fluent aqueous mixture or suspension of salts, a paste of salts, or a fused mass of salts.

Another object of the invention is to provide a flux of this kind which adheres tenaciously to the steel and which is not completely melted, burned off or otherwise injured or removed during dipping in a molten aluminum bath until it has been submerged in the molten aluminum.

A further object of the invention is to provide a flux of this kind which readily melts and disappears when an article coated with it is submerged in molten aluminum, in order to expose unoxidized surface portions of the article to the molten aluminum.

An additional object of the invention is to provide a flux of this kind which provides a substantially integral bond between aluminum and ferrous metal as well as other metals during immersion of such metals in molten aluminum.

In practicing the improved aluminum or aluminum alloy coating process, the metal to be coated, preferably ferrous metal or metal of the iron group, is first coated with an oxide reducing and air excluding coating of flux which tenaciously adheres to the metal to be treated and which does not melt or break down until the flux coated metal is immersed in a molten aluminum or aluminum alloy bath. The flux coating formed and applied according to our invention remains intact on the metal to be treated as the metal is projected, in accordance with conventional practice, into the molten aluminum or aluminum alloy bath and that part of the metal being coated immediately adjacent the surface of the bath and yet exposed to the atmosphere above the bath remains coated with flux during immersion of successive adjacent portions of the metal being treated as the latter is slowly projected into the bath.

Our improved flux may comprise a fluent aqueous mixture or suspension of certain hereinafter recited salts or it may be produced as a paste of certain salts hereinafter set forth in which a small amount of water is included as a binder. If desired, the flux may be employed in the form of a fused mass of certain salts hereinafter set

forth into which the metal to be aluminum coated may be dipped in order to deposit thereon a layer of fused salts which immediately solidify at room temperature.

5 The suspension form of the flux may be produced by mixing in 100 parts of water by weight the following proportions of salts:

|                                                       | Parts by weight |
|-------------------------------------------------------|-----------------|
| Sodium fluosilicate ( $Na_2SiF_6$ )                   | 2 to 40         |
| Potassium chloride (KCl)                              | 2 to 10         |
| Sodium chloride (NaCl)                                | 2 to 10         |
| Sodium fluoride ( $NaF$ ) or cryolite ( $Na_3AlF_6$ ) | 0.2 to 40       |

10 15 The following proportions within the above range are preferred:

|                                                       | Parts by weight |
|-------------------------------------------------------|-----------------|
| Sodium fluosilicate ( $Na_2SiF_6$ )                   | 4 to 20         |
| Potassium chloride (KCl)                              | 3 to 5          |
| Sodium chloride (NaCl)                                | 3 to 5          |
| Sodium fluoride ( $NaF$ ) or cryolite ( $Na_3AlF_6$ ) | 0.8 to 5        |

25 In the foregoing formulas, either sodium fluoride or cryolite, a common name for sodium aluminum fluoride, may be employed. The above portions of salts produce a suspension into which the ferrous or other metal parts to be aluminum coated are dipped following cleaning of them and while the flux suspension is heated to slightly under a boiling temperature. When parts are removed from the suspension, they carry with them a continuous film of the suspension which rapidly dries because of the temperature to which the suspension is heated and under the influence of the heat imparted from the suspension to the work. As the suspension dries, a substantially air impervious crust-like film of the salts of the suspension is formed on the work in a way which produces an oxide reducing and air excluding envelope about the work.

30 40 45 After the flux coating has dried, the work may be inserted in a molten bath of aluminum or aluminum alloy. The aluminum and aluminum alloy bath need not be chemically pure. The immersion of the flux coated work preferably takes place while the bath is at a temperature slightly above its melting point.

The paste type flux may be formed by mixing 50 together substantially 15 parts by weight of zinc chloride, 35 parts by weight of sodium chloride, 25 parts by weight of potassium chloride and 25 parts by weight of cryolite. Sufficient water is added to this mixture to bring the paste to a desired consistency such that it may be con-

veniently brushed or otherwise applied on to the work. The layer of flux paste is allowed to dry thoroughly before the flux paste coated work is immersed in molten aluminum in accordance with the above procedure.

The fused salt type flux preferably comprises substantially equal parts of zinc chloride, sodium chloride, potassium chloride and either sodium fluoride or cryolite, the chemical composition of which is set forth above. This mixture of salts is preferably heated to and maintained at approximately 1200° F. The work to be aluminum coated is dipped into the fused salt bath and removed and retained at atmospheric temperatures sufficiently long for the coating of fused salts to solidify. The thus coated work is then immersed in a molten aluminum or aluminum alloy bath in accordance with the above specified procedure.

It is found that work aluminum coated in accordance with the above process, by immersing it in an aluminum or aluminum alloy bath while the surfaces of the work are covered with flux coatings of any of the foregoing types, is characterized by substantially integral bonds between the metal work and the aluminum layer. All of the ingredients of the various formulas of the flux are comparatively inexpensive and readily available.

Although but several specific embodiments of our invention have been described, it is understood that various changes in the materials employed and in the sequence of steps as well as in the temperature and periods of heating may be made without departing from the spirit of our invention.

We claim:

1. A fluent aqueous flux for conditioning ferrous metal for the reception of an adherent immersion formed coating of aluminum, said flux consisting of the following substances as essential constituents and in substantially the proportions given: 100 parts by weight of water, 2 to 40 parts by weight of sodium fluosilicate, 2 to 10 parts by weight of sodium chloride, 2 to 10 parts by weight of potassium chloride and 0.2 to 40 parts by weight of sodium fluoride.

2. A fluent aqueous flux for conditioning ferrous metal for the reception of an adherent immersion formed coating of aluminum, said flux consisting of the following substances as essential constituents and in substantially the proportions given: 100 parts by weight of water, 2 to 40 parts by weight of sodium fluosilicate, 2 to 10 parts by weight of sodium chloride, 2 to 10 parts by weight of potassium chloride and 0.2 to 40 parts by weight of sodium aluminum fluoride.

3. The process of forming corrosion resisting coatings consisting essentially of aluminum on ferrous metal bodies which consists in coating the ferrous metal with an adherent fluent aqueous flux consisting of the following substances as essential constituents and in substantially the proportions given: 100 parts by weight of water, 2 to 40 parts by weight of sodium fluosilicate, 2 to 10 parts by weight of sodium chloride, 2 to 10 parts by weight of potassium chloride, and 0.2 to 40 parts by weight of a compound selected from the group consisting of sodium fluoride and sodium aluminum fluoride; forming a continuous

40  
45  
50

coating of said flux on said metal which upon drying will provide an oxide reducing and air excluding film of the salts of the flux thereon, drying said coating and immersing said flux coated metal in a molten metal bath consisting essentially of aluminum.

4. A fluent aqueous flux for conditioning ferrous metal for the reception of an adherent immersion formed coating of aluminum, said flux consisting of the following substances as essential constituents and in substantially the proportions given: 100 parts by weight of water, 2 to 40 parts by weight of sodium fluosilicate, 2 to 10 parts by weight of sodium chloride, 2 to 10 parts by weight of potassium chloride, and 0.2 to 40 parts by weight of a compound selected from the group consisting of sodium fluoride and sodium aluminum fluoride.

5. A fluent aqueous flux for conditioning ferrous metal for the reception of an adherent immersion formed coating of aluminum, said flux consisting of the following substances as essential constituents and in substantially the proportions given: 100 parts by weight of water, 4 to 20 parts by weight of sodium fluosilicate, 3 to 5 parts by weight of sodium chloride, 3 to 5 parts by weight of potassium chloride, and 0.8 to 5 parts by weight of a compound selected from the group consisting of sodium fluoride and sodium aluminum fluoride.

6. The process of forming corrosion resisting coatings consisting essentially of aluminum on ferrous metal bodies which consists in coating the ferrous metal with an adherent fluent aqueous flux consisting of the following substances as essential constituents and in substantially the proportions given: 100 parts by weight of water, 4 to 20 parts by weight of sodium fluosilicate, 3 to 5 parts by weight of sodium chloride, 3 to 5 parts by weight of potassium chloride, and 0.8 to 5 parts by weight of a compound selected from the group consisting of sodium fluoride and sodium aluminum fluoride; forming a continuous coating of said flux on said metal which upon drying will provide an oxide reducing and air excluding film of the salts of the flux thereon, drying said coating and immersing said flux coated metal in a molten metal bath consisting essentially of aluminum.

WALTER E. JOMINY.  
JOHN H. OLSON.

References Cited in the file of this patent

UNITED STATES PATENTS

| Number    | Name          | Date          |
|-----------|---------------|---------------|
| 1,653,482 | Spengler      | Dec. 20, 1927 |
| 1,941,750 | Johansson     | Jan. 2, 1934  |
| 2,101,553 | Mattsson      | Dec. 7, 1937  |
| 2,498,199 | Block         | Feb. 21, 1950 |
| 2,500,673 | Gibson        | Mar. 14, 1950 |
| 2,544,670 | Grange et al. | Mar. 13, 1951 |

FOREIGN PATENTS

| Number  | Country       | Date          |
|---------|---------------|---------------|
| 314,400 | Great Britain | July 24, 1930 |

OTHER REFERENCES

Handbook of Chemistry & Physics, 27th Ed. (1943) pages 456, 457, 458, 459, published by Chemical Rubber Publishing Co., Cleveland, Ohio.